

# UNITED STATES PATENT OFFICE.

FREDERICK MILTON JOHNSON, OF SAN FRANCISCO, CALIFORNIA.

## PROCESS OF TREATING ORES.

No. 873,943.

Specification of Letters Patent.

Patented Dec. 17, 1907.

Application filed June 3, 1904. Serial No. 211,051.

*To all whom it may concern:*

Be it known that I, FREDERICK MILTON JOHNSON, citizen of the United States, residing at San Francisco, in the county of San Francisco and State of California, have invented certain new and useful Improvements in Processes of Treating Ores, of which the following is a specification.

My invention relates to the extraction of the precious materials from ores, and especially from those ores which cannot be effectively treated by concentration, amalgamation or like processes. Such are sulfid, and pyritic and arsenical ores. Some ores of this kind yield readily to the treatment by the cyanid process, but require to be precipitated by zinc shavings in order to recover the values; and one object of my invention is to do away with the use of such zinc shavings, 20 and substitute therefor simple precipitating plates.

My process comprises broadly the mixing with the solution in the cyaniding tank of any of the soda solutions which dissolve silver, 25 preferably caustic soda, by means of which a superior action is obtained.

In treating sulfids and pyritic and arsenical ores, the ore is put into a tank containing a solution of caustic soda, and which is 30 provided with some kind of agitating device for keeping the mass stirred up and preventing settling. While in this tank and being agitated, it is subjected to the action of an electric current of high amperage and low voltage derived from any suitable source of 35 electrical energy. The result of the combined chemical and electrical actions, on ores of this character, is to remove sulfur and arsenic, to remove any iron present, to wholly 40 or partially dissolve any silver, and to effect a general decomposition of the mass which puts it in better condition for the cyaniding. After this treatment, the whole mass, without any further separation, goes directly into 45 the cyanid tank, and this explains what I previously alluded to, that the solution of caustic soda is indirectly mixed with the cyanid solution when this preliminary treatment is employed. In the cyanid tank the

gold is dissolved by the cyanid, and the caustic soda continues its solvent action on the silver, both working in harmony upon the said metals.

When the cyanid treatment has been completed, and the mass is ready for precipitation, I use, instead of the customary zinc shavings, simple plates of zinc and aluminum which are preferably bound together with copper strips. I prefer to use a flat plate of zinc between two flat plates of aluminum, riveting copper strips around the ends so as to bind all together into a single structure. I have found that with a plate of this character a perfect precipitation of both gold and silver is effected.

If the ore requires no preliminary treatment, and is placed directly in the cyanid tank, the proportion of caustic soda to cyanid should be about equal in volume. If the preliminary treatment is required, the amount of the solution of caustic soda used in the decomposing tank, should be such that when the mass is transferred to the cyanid tank, the proportion of caustic soda shall be about equal in volume to the amount of cyanid.

Heretofore, the recovery of silver by the ordinary cyanid process, has been very imperfect and unsatisfactory; only a portion of the silver being dissolved. In using the soda solution in the cyanid tank, the cyanid solution acts as heretofore on the gold, and the soda solution acts directly upon the silver, in perfect harmony with the cyanid, thereby completely dissolving both metals. In addition the two solvent elements thus combined, form a chemical solution that acts upon my plates, giving a perfect precipitation and doing away entirely with zinc shavings.

Having thus described my invention, what I claim as new and desire to secure by Letters Patent, is:

The herein-described method of treating sulfids and pyritic arsenical ores, which consists in placing the ores in a tank containing a solution of caustic soda, agitating the contents of the tank, during such agitation sub-

jecting the contents to the action of an electric current of high amperage and low voltage, then transferring the entire mass or contents of the tank to a cyanid tank and sub-  
jecting it to the action of a solution of cyanid of potassium in the presence of caustic soda, substantially as described.

In testimony whereof I have affixed my signature, in presence of two witnesses, this twenty sixth day of April 1904.

FREDERICK MILTON JOHNSON.

Witnesses:

L. W. SEELEY,  
M. R. SEELEY.